

# United States Patent [19]

Hunt, deceased

[11] Patent Number: 4,690,875

[45] Date of Patent: Sep. 1, 1987

## [54] HIGH VACUUM CAST INGOTS

[75] Inventor: Charles d'A. Hunt, deceased, late of Petaluma, Calif., by Barbara A. Hunt, executrix

[73] Assignee: Degussa Electronics Inc., Materials Division, Morgan Hill, Calif.

[21] Appl. No.: 881,218

[22] Filed: Jul. 2, 1986

### Related U.S. Application Data

[63] Continuation-in-part of Ser. No. 747,332, Jun. 21, 1985, abandoned, which is a continuation-in-part of Ser. No. 570,176, Jan. 12, 1984, Pat. No. 4,558,729.

[51] Int. Cl.<sup>4</sup> ..... B22D 25/06

[52] U.S. Cl. ..... 428/577; 428/586; 428/937; 148/425; 148/426; 148/428

[58] Field of Search ..... 164/469, 122, 46, 474, 164/462, 463, 506, 422, 494, 61; 148/31, 425, 426-429, 36-38; 428/577, 937, 586, 611

## [56] References Cited

### U.S. PATENT DOCUMENTS

- |           |         |                |          |
|-----------|---------|----------------|----------|
| 2,880,483 | 4/1959  | Hanks et al.   | 164/474  |
| 3,343,828 | 9/1967  | Hunt           | 266/34   |
| 3,367,394 | 2/1968  | Roder et al.   | 164/46   |
| 3,709,284 | 1/1973  | Hunt           | 164/281  |
| 3,723,101 | 3/1973  | Hunt           | 75/126 R |
| 3,723,102 | 3/1973  | Lowe           | 75/128 R |
| 3,764,297 | 10/1973 | Coad et al.    | 75/10    |
| 3,821,979 | 7/1974  | Paton et al.   | 164/252  |
| 3,909,921 | 10/1975 | Brooks         | 164/46   |
| 4,066,117 | 1/1978  | Clark et al.   | 164/133  |
| 4,121,647 | 10/1978 | Paton et al.   | 164/50   |
| 4,261,412 | 4/1981  | Soykan et al.  | 164/52   |
| 4,418,124 | 11/1983 | Jackson et al. | 428/678  |

### FOREIGN PATENT DOCUMENTS

58-86969 5/1983 Japan ..... 164/46

### OTHER PUBLICATIONS

Unit Processes of Extractive Metallurgy; Chapter 8 Melting, Pouring, and Solidification, pp. 226-260.

Primary Examiner—L. Dewayne Rutledge

Assistant Examiner—John J. Zimmerman

Attorney, Agent, or Firm—Fitch, Even, Tabin & Flannery

[57]

### ABSTRACT

Method and apparatus for producing a fine-grain ingot are disclosed. A feedstock stick is melted to produce a series of fully molten drops or a stream, which falls on the upper surface of an ingot being formed, to cover a portion thereof which is substantially less than the ingot's total upper surface. The mold is moved laterally with respect to the feedstock stick at a rate which is high enough so that the molten metal impinges upon different portions of the ingot's upper surface but which is low enough to prevent a substantial centrifugally outward flow of the metal impinging on the upper surface of the ingot. The molten metal melt rate is so selected that the impact region on the ingot's upper surface is at or below the solidus temperature of the alloy and above a temperature at which metallurgical bonding with the successive impinging metal can occur. The resulting ingot is characterized by a uniform transverse grain size in the range of ASTM 3 to 9 and a uniform longitudinal grain size of at least equal to the transverse dimension. The ingot is further characterized by a subgranular structure of substantially equiaxed cells having an average diameter of between about 20  $\mu\text{m}$  and about 80  $\mu\text{m}$ . The ingot is substantially 100% dense, has less than 5 ppm total oxygen content and less than one ppm oxygen as insoluble oxide.

15 Claims, 6 Drawing Figures





FIG. I



FIG. 2



FIG. 4



FIG. 3



FIG. 5



FIG. 6

## HIGH VACUUM CAST INGOTS

## BACKGROUND AND SUMMARY

This application is a continuation-in part of application Ser. No. 747,332, filed June 21, 1985, now abandoned, which was a continuation-in-part of application Ser. No. 570,176, filed Jan. 12, 1984 now U.S. Pat. No. 4,558,729.

The present invention relates to metal casting, and more particularly, to improvements in high vacuum cast ingots.

The production of ingots by continuous casting in high vacuum is well known in the prior art. Generally, a continuous casting process employs a mold having a cooled outer wall and a movable bottom, or plug. Molten metal is poured into the top of the mold in a vacuum enclosure. As the metal solidifies, it is drawn downwardly by the plug while, at the same time, additional molten metal is poured into the mold at the top.

Because heat loss from the ingot in this type of continuous casting process occurs primarily at the cooled mold walls and downwardly through the solidified portion of the ingot, the solidification of the molten metal in the newly poured ingot occurs at relatively low rates. For example, movement of the liquid-solid interface at rates slower than approximately 1/10 inch per minute in the central regions of the ingot is typical. For many materials, and particularly more complex alloys, the relatively slow solidification rate is accompanied by the growth of dendritic crystals having large arm spacings, and by significant segregation of various alloy constituents in the regions between the dendritic arms.

Conventionally cast ingots having dendritic crystal and segregation imperfections of the type mentioned above usually require annealing prior to being subjected to mechanical hotworking operations such as rolling and forging. For example, heating to temperatures slightly below the alloy's solidus temperature for periods of up to 24 to 36 hours is typical. Even then, hot working of conventionally cast ingots of many complex alloys may be accompanied by so much surface cracking that some of these ingots are considered to be unworkable.

Another problem associated with conventional continuous casting processes known in the prior art is the formation of ruptures in an ingot sidewall during ingot casting. The ruptures, or so-called hot tears, are formed by frictional forces between the ingot and mold when the ingot is lowered in the mold before its sidewall regions have cooled sufficiently. For most purposes, hot tears constitute an unacceptable sidewall condition where further processing of the ingot is required.

A number of casting techniques for producing ingots which have reduced hot-tear and segregation problems have been proposed. Some newer casting techniques are designed particularly for the production of high quality, ultrahigh-strength alloy ingots which are suitable for rolling, forging or the like. U.S. Pat. No. 3,709,284, discloses a continuous casting method in which a water-cooled ram or plug periodically engages the top of the ingot during casting, to cool the ingot from its upper surface. The method involves contacting the cooling plug with each newly poured molten-metal layer, which may have a thickness of about 1/16 inch. Electron beam heating is used to heat the ingot's upper sur-

face between solidification operations to assure good bonding between the successive layers.

As the plug makes repeated contact with the upper surface of the newly poured increments, it begins to collect a surface contamination coating or deposit which is formed, in part, from metal vapors from the molten alloy. Since the coating which collects on the plug has a different composition than that of the alloy itself, the plug must be cleaned periodically to prevent the material from being introduced into the ingot melt. The need to keep the plug surface clean adds to the complexity and expense of the operation, and unless the plug is kept completely free of vapor coatings, some contamination of the ingot will occur. This process, therefore, is best suited for high-strength steels and other alloys that do not need to be ultra-clean.

Because of the above-mentioned problems, parts forged from high vacuum cast ingots have heretofore been unsatisfactory for many applications. This is particularly true with respect to parts which are subject to repeated cycling at relatively high temperatures (e.g. 1300°-1400° F.). This is also particularly true with so-called super alloys of the type often used in aircraft engines and the like.

Ultrahigh-strength alloys having a fine-grain crystalline structure may be produced by powder metallurgy. This approach is common in the manufacture of many types of aircraft engine parts. The powdered alloy can be converted to the equivalent of a billet by means of conventional hot pressing techniques, and such billets can then be converted to forged parts that exhibit excellent mechanical properties. However, powder metallurgy methods typically provide a relatively low yield of usable powder, and thus material costs are high.

Additionally it is difficult to prevent damaging impurities from contaminating the powder. Consequently, manufacturing costs using powder metallurgy are often undesirably high.

To avoid the high manufacturing costs associated with the use of powder metallurgy, attempts have continued to provide ingot casting processes which produce ingots of high cleanliness and adequate grain refinement and uniformity. One such prior art process is shown and described in U.S. Pat. No. 4,261,412. In the process described, a spray of molten droplets from a pair of consumable electrodes, heated by vacuum arc melting, drips onto the upper surface of an ingot being formed in a spinning mold. As the molten drops hit the ingot surface, near the center of the spinning mold, the metal spreads out in a thin layer which covers the upper surface of the ingot.

Ingots produced by the spinning mold process may lack a truly fine grain size. Rather, such ingots typically achieve grain sizes at or exceeding ASTM 3-4. The heated material which drops onto the ingot usually does not reach the liquidus temperature, and therefore the thin layers forming the ingot contain unmelted solid particles which can seed larger grains in the solidified ingot. The need for relatively high rotational speeds in this process also introduces significant mechanical complexity to the apparatus.

Another prior art casting process is known as spray casting. For example, in U.S. Pat. No. 4,066,177, Clark et al., a process is disclosed in which an atomized metal stream is directed into a mold by using jets of a supersonic inert gas. Fine grained (within the range of 10-40 microns) cast metal bodies are produced containing average densities of the order of 95% of theoretical and

with oxygen content of the order of 26 ppm (less than half that of conventional powder metallurgy ingots). Oxygen content is reported as low as 9 ppm.

Despite the significant grain refinement achievable by the plasma spray casting technique, ingots achieved by such process have been less than desirable in terms of their insoluble oxide content and their density in the as-cast condition. The presence of insoluble oxides at levels greater than one part per million (ppm) can seriously affect the low cycle fatigue properties of many super alloys. Moreover, although plasma spray cast ingots are typically closer to theoretical density of the alloy in the as-cast condition, they are still lower in density than ideal for purposes of forging.

It is a general object of the present invention to provide improved fine-grain, high-strength alloy ingots.

A more specific object of the invention is to provide a high-strength iron, nickel or cobalt-based ingot which can be hot rolled or forged directly without the need for extensive prior heat treating of the ingot.

A related object of the invention is to provide a vacuum cast ingot that has well distributed segregates and has less than about one ppm oxygen content in the form of insoluble oxides.

Yet another object of the invention is to provide a continuous vacuum cast ingot of relatively large diameter, i.e., substantially greater than 6 to 8 inches (15 cm to 20 cm), which is of high purity and has a uniform and fine segregate distribution.

The objects of the invention are met by providing a vacuum cast, high-strength iron, nickel or cobalt-based alloy ingot wherein the average diameter of the grains when viewed on a surface cut perpendicular to the longitudinal axis of the ingot is between about 50  $\mu\text{m}$  and about 500  $\mu\text{m}$ , and wherein the average diameter of the grains when viewed on a surface cut parallel to the longitudinal axis of the ingot is at least equal to the said perpendicular diameter. The ingot is further characterized by a subgranular structure of substantially equiaxed cells having an average diameter between about 20  $\mu\text{m}$  and about 80  $\mu\text{m}$ . The ingot is substantially one hundred percent dense and has less than 5 ppm total oxygen content and less than 1 ppm oxygen as insoluble oxide.

#### BRIEF DESCRIPTION OF THE DRAWINGS

FIG. 1 is a diagrammatic sectional view of a high vacuum drop-casting apparatus for use in producing ingots according to the invention;

FIG. 2 is a sectional view of a mold in the apparatus, taken generally along line 2-2 in FIG. 1, showing the upper surface of an ingot in the mold during the formation of an ingot surface layer;

FIG. 3 is a sectional view taken generally along line 3-3 in FIG. 2, illustrating the overlapping of successive layers in the ingot being formed;

FIG. 4 shows an alternative embodiment of the apparatus, where the mold of FIG. 1 is equipped with an inner curved wall member used in forming an ingot having a hollow cylindrical interior;

FIG. 5 is a transverse cross sectional photomicrograph, magnified 500 times, of an ingot of the invention; and,

FIG. 6 is an axial cross sectional photograph, at unity magnification, of an ingot of the invention.

#### DETAILED DESCRIPTION OF THE INVENTION

FIG. 1 shows, in diagrammatic form, an apparatus 10 for forming a fine-grain alloy ingot according to the invention. The apparatus 10 includes a vacuum-tight enclosure or furnace 12 which can be evacuated to a desired pressure, preferably less than about  $10^{-3}$  Torr, by one or more vacuum pumps, such as a pump 14.

A feedstock support 16 in the apparatus is adapted to support a feedstock stick 18, the lower end portion of which is seen in the figure. The support is constructed to advance the stick in a downward direction in the figure, as the heated stick's lower end is depleted during ingot formation. Preferably, the support is designed to maintain the lower end of the stick a vertical distance between about 4 and 12 inches (10-30 cm) above the upper surface of the ingot being formed, and is constructed to rotate the stick about its central vertical axis, shown by dash-dot line 19.

One or more electron beam guns, such as the gun 20, are provided for melting the lower end of the feedstock stick. The electron gun(s) may be either the self-accelerated or work-accelerated type, and may be mounted in the enclosure for adjustable movement to position the beam(s) at a desired position with respect to the support 16. Magnetic deflection of the beam may also be used to adjust its position relative to the support 16. Magnetic deflection means are built into the structure of electron guns commercially available from Leybold-Heraeus of Hanau, West Germany, and the von Ardenne Institute of Dresden, East Germany.

A continuous casting mold 22 in the apparatus 10 includes a cylindrical housing 24 having coolant passages 25 in the walls thereof for circulation of a suitable coolant to withdraw heat being formed in the mold. A water-cooled plug 26 of suitable material is provided inside the housing to form the lower support for an ingot formed in the mold. The plug is supported on a plate 28 which is connected by a rod 30 to a piston 32 in a conventional hydraulic cylinder 34. The vertical position of plug 26 is controlled conventionally by suitable hydraulic control of the cylinder 34. The cylinder is rigidly attached at its upper end to a lower base 36 in the mold housing, with the rod 30 being slideably received through a central opening in the base. Of course, other control means could be used to position the plate 28, such as a ball screw drive system.

The apparatus 10 includes means for producing relative movement between the mold 22 and the support 16. This movement allows molten metal from the heated feedstock stick to impinge upon different portions of the upper surface of the ingot being formed in the mold, in a manner to be described. To produce such movement, the apparatus 10 includes a cart 38 on which the mold 22 (including the mold housing 24 and attached cylinder 34) is mounted for rotation about the mold's vertical axis. Cart-mounting structure, indicated generally at 40, mounts the cart 38 for reciprocal lateral motion in the directions indicated by the arrow 41 in the figure.

The cart 38 includes an outer support member 42 which is carried on a structure 40, and which defines an inner circular bearing surface 44 in the cart. An inner annular member 46 in the cart is mounted within the inner bearing surface of the member 42, by bearing balls 48, for rotational movement with respect to the member 42 about its central vertical axis, which coincides with the central axis of the mold 22. A suitable hydraulic

system (not shown) is operable to produce a selected-speed rotation of the inner member 46 with respect to the outer member 42, for a purpose to be described.

The mold 22, and particularly the cylinder 34 therein, is rigidly mounted in a central opening in the member 46 for rotation therewith about the mold's vertical axis, indicated by the dash-dot line 49 in the figure. It can be appreciated that the just-described mold, including the housing 24 and the plug 26, which is vertically movable therein, is rotated as a unit with the inner member 46.

The mounting structure 40 generally includes a pair of parallel tracks, such as the track 50, mounted on and extending between opposed walls in the enclosure 12. The cart 38, and particularly the outer member 42 therein, is carried on the tracks by roller balls or the like, such as balls 51, for shifting movement along the tracks. The roller balls 51 ride in suitable grooves formed in the lower surface of the member 42 and in the mounting structure tracks. The groove 53 in the track 50 is seen in FIG. 1. It is noted that the cylinder 34, a portion of which extends below the tracks, is disposed between the two tracks in the mounting structure 40.

Shifting means for moving the cart and attached mold selectively to the right or left in the figure is provided by a second hydraulic cylinder 52 mounted on one of the enclosure walls, as shown, and connected to the cart by a rod 54. For purpose of illustration, the apparatus will be assumed to have a mold radius, as measured by the radial distance between the mold's center axis and its inner wall, of 6 inches (15 cm). With the cylinder in its retracted position, as shown in FIG. 1, the mold is positioned with its central axis 49 offset from the drip axis 19 by a radial distance  $r$ , as shown. The significance of  $r$ , which is here assumed to equal one inch or 2.5 cm, will become clear below. With mid extension of the cylinder 52, the mold is moved toward the left in the figure a distance  $2r$  (2 inches or 5 cm), to a position where the drip axis 19 is spaced a radial distance  $3r$  (three inches 7.5 cm) from the mold's central axis. Movement of the cylinder to its fully extended position carries the mold 20 an additional distance  $2r$  to the left in the figure to a position where the mold drip axis 19 is spaced a radial distance  $5r$  (five inches or 12.5 cm) from the center axis of the mold.

Completing the description of what is shown in FIG. 1, the apparatus 10 includes a second electron gun system, represented here by an electron gun 56, which is operable to provide electron-beam heating of the upper surface of the ingot being formed in the mold 22. The one or more electron guns, such as gun 56, in the electron-gun system are substantially identical to that of the above-described gun 20, and are movable either for electron-beam scanning of the upper surface of the ingot being formed, or for directing the beam(s) at selected positions on the mold's upper surface. Adding heat by electron beam to the top surface of the ingot is generally undesirable, except at the end of a run, when it is sometimes desirable to reduce the rate of cooling of the top surface of the ingot to prevent shallow cracks from developing there.

Production rate is limited by the rate of heat loss from the top surface of the ingot during the thin-layer casting operation. Therefore the impingement of electron beams on this surface during the casting operation constitutes an undesirable heat source that reduces the maximum production rate possible in this type of operation.

The operation of the apparatus 10, as it is used to produce the ingots of the invention, will now be de-

scribed. The feedstock stick placed in the support 16 includes a stick or cylinder of the alloy metal from which the ingot is formed. The present invention is particularly useful in connection with nickel- or cobalt-based alloys containing at least about 50% nickel or cobalt, respectively, and between about 10% and 20% chromium. Alloys of this type that contain significant fractions of aluminum and titanium, as well as higher melting point elements such as niobium, molybdenum, and tungsten, are known as superalloys, being characterized by relatively broad liquidus-solidus temperature ranges, typically between about 120° F. and 300° F. (65° C. and 150° C.). Such alloys may contain one or more elements selected from the group consisting of niobium, molybdenum, tungsten, yttrium, tantalum, hafnium, zirconium, and vanadium.

The electron-beam gun or guns in the feedstock beam heating system, such as the gun 20, are aimed at the lower end of the feedstock stick to produce fully molten drops at the bar's lower end. The electron beam, or beams, preferably make a 10° to 30° angle with the horizontal, as shown. The desired feed rate is established by setting the rate of downward movement of the feedstock stick in the support 16. The total electron-beam power is adjusted to a level about 10% to 30% greater than that necessary to melt completely the lower end of the feedstock stick as it moves downward into the beam. By way of example, a beam power of about one-fifth kilowatt total beam power per pound of melt per hour has been used for nickel-based superalloys. This total beam energy may be supplied by one electron beam gun aimed at one side of the feedstock stick, as shown in FIG. 1, or by a series of guns arrayed within the enclosure to irradiate the feedstock bar's lower end from different sides. It is generally necessary to rotate the stick in the support 16, about the stick's central vertical axis, to produce even heating at the stick's end, and to insure dripping along the stick's vertical axis 19. This axis is also referred to herein as the drip axis.

When molten metal hits the upper surface of an ingot being formed in the mold, it forms a film-like spatter which covers a portion of the upper ingot surface that is substantially less than the total upper ingot surface. Fully molten metal of a superalloy of the type described above, falling a distance of between about 4 and 12 inches (10-30 cm) from the stick to the upper surface of the mold, typically forms a roughly circular spatter having a diameter of between about 1.5 and 2.5 inches (3.8 and 6.2 cm), and a fairly uniform spatter thickness of between about 15 and 30 mils (0.04 to 0.08 mm). For purposes of the present discussion, the average spatter will be assumed to have a surface dimension of about 2 to 2.5 inches (5 to 6.2 cm) and a thickness of about 20 mils (0.05 mm). The radius of the spatter is thus about 1 to 1.25 inch, which is equal to or greater than  $r$ .

According to an important feature of practicing the process, the mold 22 is moved laterally with respect to the drip axis 19, at a rate which is high enough to lay down a close-packed array of spatters which form each of the successive ingot layers. Lateral movement of the mold includes both translational movement (in a left-right direction in FIG. 1) and rotational movement about the mold axis 49. The relative movement is low enough, however, so as to prevent a substantial centrifugally outward flow of molten metal impinging on the top surface of the ingot. This avoids uneven buildup of metal on the ingot which is significant in preventing

limitations on production rates due to excessive buildup at the periphery of the ingot.

Describing a typical operation of the apparatus 10 in producing such a spatter array, with the mold in the lateral position shown in FIG. 1, a molten drop from the feedstock stick forms a substantially circular spatter, such as the spatter 62 seen in dotted outline in FIG. 2, extending from the center of the mold radially outwardly about 2.25 inches. By rotating the mold in a specified direction, e.g., counterclockwise in FIG. 2, at a selected speed, the next drop falling on the ingot forms a spatter, such as spatter 64, which is adjacent the previously formed spatter 62.

Spatter drops can overlap by as much as about 70% to 85% (diametrically). The critical factor is not the overlap or lack of overlap but rather the average rate of vertical buildup of solidified metal. For super alloys, this average rate of vertical buildup cannot exceed about 0.4 inches (1 cm) per minute without the occurrence of molten areas on top of the ingot, with attendant substantial increase in grain size. Also if the rate of lateral movement is so slow that the short-time average of local buildup rates exceeds about 0.4 inches (1 cm) per minute for periods exceeding about 10 seconds, then the surface of the local areas upon which the drops are impinging will remain molten for periods longer than about one second, with resulting local increase in grain size of the solidified ingot. Some degree of overlap is generally desirable to obtain a smoother ingot side wall and to minimize the possible occurrence of unfilled areas at the borders between splatters. Too much overlap, however, can create the situation noted above concerning excessive short-time average rates of local buildup. Thus, for any feed rate, there is a particular average rate of ingot buildup that results; and that rate (average) must not exceed about 0.4 inches (1 cm) per minute. Then, the cycle repeat time cannot exceed about 100 seconds without having the possibility of inadequate bonding between layers.

In addition to following the aforesaid limitations on overall ingot buildup rate, care must be taken to avoid localized pooling of molten metal. Such pooling results in undesirable non-uniformity of grain structure. It is preferred that the local short-time buildup not exceed 0.4 inches per minute for a period exceeding about 10 seconds.

Continued rotation of the mold, through substantially one rotation in the direction indicated in FIG. 2, causes the next two molten drops to form spatters 66, 68. As seen, these four spatters 62, 64, 66, 68 form a nearly continuous layer or covering extending approximately 2 to 2.25 inches radially outwardly from the center of the mold.

The mold is now shifted translationally, by activation of the cylinder 52, to a position where the axis 19 is offset about 3 inches (7½ cm) to the right of the axis 49 in FIG. 1. With the mold so positioned, the next impinging drop then will form a spatter, such as the spatter 70, seen in FIG. 2, whose center is about 3 inches (7½ cm) from the center of the mold. The mold is again rotated in the specified direction, at a now-slower rotational speed, through substantially one rotation, to produce a second annular "ring" of spatters, including the spatters 70, 72, 74, which extend the surface covering on the upper surface of the ingot a distance about 4 to 4.25 inches from the center of the mold.

Finally, the mold is moved translationally by full extension of the cylinder 52, to the position where axis

19 is offset about 5 inches (12½ cm) from the center of axis 49. The mold is then rotated at a further reduced speed, through substantially one rotation, to lay down a outer annular ring of spatters, including the spatters 76, and 78, to form a new ingot layer having a thickness of about 20 mils (0.05 mm).

The mold rotational speeds required to attain the spatter pattern just described depend, of course, on the drip rate of molten drops impinging on the mold upper surface. The drip rate is an important parameter in the practice of the invention and will be discussed in detail below. For purposes of the present discussion, the drip rate will be assumed to be about 5 drips per second. To form the innermost ring of spatters, composed of four or more spatters, the mold must be rotated at about 60 rpm or less, allowing deposit of the first four drops in 4/5 second or longer.

The approximately 12 or more spatters forming the central annular region, including the spatters 70, 72, 74, are deposited in the next 2 and 2/5 seconds or longer, requiring a mold rotational speed of about 23 rpm or less. Finally, the approximately 20 or more spatters forming the outer circle are deposited in approximately 4 or more seconds, requiring a mold rotational speed of about 15 rpm or less.

Thus, as the mold is moved in a right-to-left direction in the figure to form increasing-radius annuli or rings of spatters, the rotational speed of the mold is progressively decreased. After completing the cycle, the mold is retracted to its initial position shown in FIG. 1 and the procedure is repeated, to build up increasing ingot layers. Periodically, the plug 26 in the mold is retracted to accommodate the buildup of ingot layers in the mold. The ingot being formed in the mold 22 is indicated at 79 in FIG. 1.

As seen in FIG. 2, the top layer in the ingot, which is formed as an array of spatters as just described, is formed of thin overlapping spatters. The edges of these spatters form depressions in the ingot's upper surface which tend to be filled and average out to a fairly level surface as the next spatter layers are formed, as will now be illustrated with reference to FIG. 3. Spatters 80, 82, 84, which are shown enlarged and in exaggerated cross-sectional thickness in FIG. 3, represent spatters which were laid down in a previous layering operation of the type just described. As the next layer of spatters, including spatters 86, 88, is laid down, molten spatter material flows into and fills the edge regions in the immediately preceding layer, as shown. Edge fusion of splatters occurs naturally, without the need for electron beam assistance.

The rate at which successive layers are formed is such that the drop impact region on the ingot's upper surface is at or below the solidus temperature of the ingot alloy and above a temperature at which metallurgical bonding with the successive impinging drops can occur. Empirically, for the super alloys of the type described herein, the cycle rate—defined herein as the rate at which successive drops impinge on substantially the same surface portion of the ingot's upper surface is between about 3 and about 100 seconds. If the rate of successive impingement of molten drops at a given location is more than about one every three seconds, a molten pool begins to collect in the ingot upper surface, leading to slower solidification and a coarser grain size in the ingot being formed. At a cycle rate of more than about 100 seconds, good metallurgical bonding between successive overlaid spatters may not be achieved. For

alloys of the type mentioned, good metallurgical bonding occurs where the impact region is between about 50° F. and 200° F. (28° C. and 110° C.) below the solidus temperature of the ingot alloy.

Photomicrographic examination has shown that there is some growth of dendrites vertically across the boundary between spatters. This dendritic growth tends to be more pronounced at shorter repeat cycle times and less pronounced at longer repeat times. Although the presence or absence of dendritic growth across the boundary between spatters is not presently known to have an affect on the properties of the material, such dendritic growth clearly establishes that there is substantial integrity in the bond between successive spatters.

The cycle rate defines the time required to deposit all of the spatters forming one layer. Therefore, the cycle rate will depend on the drip rate of molten drops from the feedstock stick. By way of illustration, a 12-inch diameter ingot surface as seen in FIG. 2 may be covered by approximately 36-42, 2 to 2.5 inch diameter spatters with overlap sufficient to leave no uncovered areas. At a drip rate of about 7 drops per second, the entire surface of the ingot can be covered approximately every 6 seconds, the cycle rate of operation.

By way of further example, a drip rate of 0.7 drops per second (1/9 the above rate) builds up a 4 inch diameter ingot approximately at a rate of about 0.2 inches (0.5 cm) per minute, as would a 6 second cycle on a 12 inch ingot.

Of interest here is the fact that a feed rate of 12 drips per second would give a buildup rate of about 0.4 inches (1 cm) per second, the estimated maximum possible upper limit of production. A cycle time of 6 seconds corresponds to about 50% overlap of droplets, which is satisfactory. The local short-time average spatter impingement time is still quite brief (nowhere near the 10 second limit).

The production of a fine-grain ingot having a hollow cylindrical interior can be accomplished with minor modifications of the apparatus and method just described. Fragmentary portions of a mold used in forming such an ingot are shown in FIG. 4. As seen, the mold includes, in addition to the cylindrical housing 24 and plug 26 described with reference to FIG. 1, an inner water-cooled mold member 90 defining an arcuate outer surface 92 which, with the member mounted in the mold housing 24, is substantially concentric with the interior of the housing walls. The mold member preferably has an arcuate expanse of between about 10° and 20°, and is tapered about 1° to 2° on progressing upwardly to compensate for shrinkage of the ingot's hollow interior as the ingot cools. The member's outer surface is provided with a hard surface, for example, a hard chrome plating. The mold member is mounted in the upper portion of the mold housing for shifting with the mold in the reciprocal left/right directions in the figure, but remains stationary with respect to the rotational movement of the mold, and also with respect to vertical movement of the plug 26.

In operation, the mold is initially positioned to place the outer surface of the member 90 between the drip axis and the mold's rotational axis, such that the spatter formed from a molten drop will abut and be defined radially inwardly by the member's outer surface. Continued rotation of the mold and deposition of spatters adjacent the mold member results in an annular spatter layer having a circular inner edge. The mold is then moved translationally, as described above, to form addi-

tional greater-diameter annular rings required to build up each ingot layer. As the ingot layers are formed, the plug 26 is retracted to lower the ingot in the mold, but still keeping the upper surface of the ingot above or at the level of the lower surface of the mold member. It can be appreciated that continued layer buildup in this fashion results in an ingot having a hollow cylindrical interior, shown here at 94. The ingot formed has a grain structure which is substantially identical to that in the solid ingot described above. A hollow ingot can also be cast without using an inner mold section. The inner surface is, of course, quite rough, in this case; and the annular wall thickness cannot be less than about 2 inches, the diameter of the spatters.

Ingots of the invention have a characteristic microstructure which is not present in ingots known in the prior art. A grain in the metallurgical sense is an area with the same undisturbed crystallographic orientation. This area is enclosed by a grain boundary, where the orientation changes either angularly or rotationally, or both. Some concentration of segregates typically exists at the grain boundaries. In the alloy of the present invention, as cast, the average diameter of the grains when viewed on a surface cut perpendicular to the longitudinal axis of the ingot (transverse dimension) is between about 50  $\mu\text{m}$  and about 500  $\mu\text{m}$ . On the other hand, the average diameter of the grains when viewed on a surface cut parallel to the longitudinal axis of the ingot (longitudinal dimension) will vary depending upon the repeat cycle time used in casting the ingot. This variation can range from about the same size as viewed on the perpendicular surface (an aspect ratio of 1) to as long as 25 millimeters (an aspect ratio of 500).

By way of example, at a repeat cycle time of 6 seconds, the grains are typically quite columnar, having a very high length-to-diameter (aspect) ratio. Typical under such conditions is a transverse grain size of about 100  $\mu\text{m}$  to about 500  $\mu\text{m}$  and a longitudinal grain size of 1 mm to about 20 mm. By contrast second repeat cycle time will typically produce transverse grain diameters of about 100  $\mu\text{m}$  to about 500  $\mu\text{m}$  with longitudinal grain size ranges from about 1 mm to about 5 mm. By further contrast, at a 60 second repeat cycle time, the grains are typically only slightly columnar, having a transverse dimension of from about 100  $\mu\text{m}$  to about 300  $\mu\text{m}$  and a grain longitudinal size of about 0.5 mm to about 2.5 mm.

A further unique characteristic of the microstructure of the alloy of the present invention in the as-cast condition is the presence of sub-granular units, typically known metallurgically as cells. A cell is a segregation pattern, due to the way in which the material solidifies. In the present invention, the cell size is sufficiently small that the segregates are essentially uniformly dispersed throughout the material. The material therefore can be forged directly in the as-cast condition, without the necessity of heat treatment in order to homogenize the segregates. This cellular microstructure, in the alloy of the invention, is substantially uniform despite variation in repeat cycle time. The cells are equiaxed and have an average diameter of between about 20  $\mu\text{m}$  and about 60  $\mu\text{m}$ .

The microstructure of the invention can be obtained even in connection with very large diameter ingots, up to and exceeding 50 centimeters in diameter. Referring to FIG. 5, a cross-sectional photomicrograph, magnified 500 times, of an ingot according to the invention is shown. The grain sizes represented are in the character-

istic 5 to 7 ASTM range, typically between about 50 and 80 microns. The larger objects visible in the photomicrograph are solidification segregates which essentially disappear during the working and annealing cycles used to convert the ingot to wrought forms. Grain structures and segregate patterns of this fineness and uniformity are not achievable by any known prior art techniques except the powder metallurgy and plasma spray techniques mentioned above.

Unlike typical grain structures achieved in powder metallurgy and plasma spraying, however, the grains of the ingot of the present invention are not symmetrical. Rather, as mentioned above, the grains in the axial direction of the ingot tend to grow longitudinally with some growing through the boundaries of the various layers or arrays of spatters, typically reaching a length in the range of 0.05 to 25 millimeters measured parallel to the longitudinal axis of the ingot. The longitudinal grains, as may be seen in FIG. 6, are oriented substantially parallel to the axis of the ingot, which is the vertical direction in the figure. Although the grains are substantially larger in the axial dimension or direction of the ingot than in the transverse direction, this factor does not appear to detrimentally affect the workability of the ingot. This unusual microstructure, characterized by fine and uniform grain refinement in the transverse direction and elongated grain dimension and alignment in the axial direction is not present in any known prior art structures. The aspect ratios (average length:average diameter) of the grains present in the ingots of the invention are typically in the range of about 1 to about 600.

As mentioned earlier, the ingots of the invention, due to their grain refinement and uniformity, are capable of being forged or hot-rolled directly without the need for extensive prior heat treatment. This is true even of characteristically difficult to work alloys such as the so-called superalloys. The ability to hot-roll or forge directly from the ingot after vacuum casting is a result of the low number and fine distribution of solidification segregates, and represents a significant improvement over known prior art techniques inasmuch as substantial cost saving results.

Ingots having diameters of 8 inches (20 cm) up to 20 inches (50 cm) or larger, and/or hollow interior ingots, 45 may be produced having the characteristics of the invention.

The following examples are illustrative of methods for producing the ingots of the invention, but are not intended to limit the scope thereof.

#### EXAMPLE I

An ingot of nickel-base superalloy was cast according to the foregoing described method, using electron beam refined feed stock, of the composition "GMR 235" (General Motors Research 235).

The feed stock was 3 inches (7.5 cm) diameter and 8 inches (20 cm) long. It was rotated at a rate of about 5 r.p.m. and fed downward at a rate that gave fully molten electron beam melted drops at a rate of 0.8 drops per second. The ingot buildup rate was about 0.2 (0.08 cm) per minute.

The top of the ingot being formed was maintained at a height that caused a drop height of about 4 inches (10 cm).

The ingot was rotated at a rate of about 5 r.p.m., the vertical axis of rotation displaced about 8 of an inch (2 cm) laterally from the vertical axis of rotation of the

feed stock (the axis of dripping, also, of course). The spatters overlapped about 50% diametrically.

No external mold surface was used, the ingot O.D. being determined by the solidification of the spatters. The rough O.D. of the resulting ingot was about 4 inches (10 cm). The roughness was about  $\frac{1}{8}$  inch (0.05 cm) deep and was removed by machining the ingot on a lathe to obtain a smooth ingot, about 5 inches (12 cm) long. The transverse grain size was ASTM 5 to 7, and the longitudinal section showed that the grains parallel to the ingot axis were about 1 mm to 10 mm long and did not reflect any grain growth phenomena affected by the layer interfaces, which were 0.020 inch (0.008 cm) thick.

#### EXAMPLE II

The experiment of Example I was repeated, except the drip height was 8 inches (20 cm). The conditions were otherwise the same, and the results were also the same.

#### EXAMPLE III

The experiment of Example I was repeated, except that the drip axis and the ingot rotation axis were displaced about  $1\frac{1}{4}$  inches. A hollow ingot with a rough hole along the central axis was cast. The internal and external roughnesses were each about  $\frac{1}{8}$  inch (0.05 cm) deep. The hole was about  $\frac{1}{2}$  inch (1.25 cm) diameter rough and about  $\frac{3}{4}$  inch (1.8 cm) diameter as smooth-machined. Grain structure was the same as in the solid ingots.

#### EXAMPLE IV

A larger ingot of nickel-base superalloy could be cast as follows:

Using a drip rate of about 2.4 drops per second and a drip height of about 8 inches (20 cm), the ingot is rotated alternately at axis displacements of about 1 inch (2.5 cm) and about 3 inches (7.5 cm) with one revolution at each radius for each dual-radius cycle. The rate of rotation at the one inch (2.5 cm) radius is 15 r.p.m., and 5 r.p.m. at the large radius.

An external water-cooled mold about 8 inches (20 cm) diameter would define the outer surface, which would have a roughness of about 1/16 of an inch (0.025 cm).

The ingot buildup rate would be about 0.2 inch (0.08 cm) per minute. The ingot grain structure would be the same as in the smaller ingots, and would be relatively uniform from edge to center and from top to bottom.

#### EXAMPLE V

A high strength alloy steel ingot (e.g. type 4340 steel) could be cast in the same apparatus and under the same conditions as for the nickel-base superalloy of Example IV. Grain size and shape would be approximately the same as for the superalloy.

#### EXAMPLE VI

Superalloy Rene' 95 (TM) was cast into a four inch square cross section mold using a 0.25 inch/min (0.635 cm/min) build-up rate. A 60 second repeat cycle time was used with a drop height of about 6 inches (15 cm) in a rectangular pattern of drips at 90-95% "overlap". Grain size was about 150  $\mu$ m transverse and about 2 mm longitudinal. Cells were equiaxed and about 30  $\mu$ m dia.

## EXAMPLE VII

Example VI was repeated except that a 4"  $\times$  12" cross section was cast using the same build-up rate and a 20 second repeat cycle time. Grain structure was more equiaxed than Example I (6 second repeat) and more columnar than Example VI (60 second repeat). Cell sizes in all superalloy examples were generally similar.

The ingots of the invention are particularly suited, in the case of superalloys, for the manufacture of parts which require good fatigue strength at high temperature. For example, many rotary parts in aircraft engines are repeatedly cycled at high temperatures, subjecting them to the possibility of failure as a result of low cycle fatigue. When such failure does occur, the cause is typically the presence of microscopic oxide inclusions, usually aluminum oxide or, sometimes, titanium oxide, since aluminum and titanium are common components of superalloys. Some alloy components, such as columbium and tantalum, form acceptable oxides because these oxides are in a soluble phase which does not segregate during casting or further manufacturing of the part. Oxides which do segregate are referred to as insoluble oxides and are not tolerable in many applications in amounts greater than one ppm oxygen. Oxide contamination can occur as a result of improper isolation or handling of powders, contamination of vacuum chambers, and contamination from crucible or tundish materials used to contain molten alloys. Due to the simplicity of the process by which the ingots of the invention are made, electron beam melted starting materials having low insoluble oxides may be utilized and further contamination is readily avoided. Accordingly, the oxide content of the ingots of the invention can be maintained at the desired low levels.

It has been discovered that the ingots of the invention are of very high and uniform density in the as-cast condition. Density measurements of ingots of the invention indicate that their density is equal to or in excess of 99.5% of the theoretical density of the alloy of which they are composed. This is significantly better than densities achievable with powder metallurgy techniques, and is also significantly better than densities consistently achievable with plasma spray techniques. As a consequence of the high density achieved in the as-cast condition, the ingots of the invention are readily forgeable for ease in fabricating parts.

It may be seen, therefore, that the ingots of the invention possess excellent density and extremely low insoluble oxide content, setting them apart from many prior art materials in both low cycle fatigue strength and ductility. In addition, the ingots of the invention possess a unique microstructure, a sort of identifying signature, wherein the cell size remains extremely fine, even though the grain size and aspect ratio may vary. Characteristically, in ingots of the invention, the aspect ratio (i.e. the ratio of average length to average diameter) of the grains is in the range of about 1 to about 600.

While preferred embodiments of the invention have been described herein, it will be apparent to those skilled in the art that various modifications and changes may be made in the invention without departing from the scope thereof, as defined by the following claims.

What is claimed is:

1. A vacuum cast high strength iron, nickel or cobalt based alloy ingot wherein the average as cast diameter of the grains when viewed on a surface cut perpendicular to the longitudinal axis of the ingot is between about

50  $\mu\text{m}$  and about 500  $\mu\text{m}$ , and wherein the average as cast diameter of the grains when viewed on a surface cut parallel to the longitudinal axis of the ingot is at least equal to the said perpendicular diameter,

said ingot being further characterized by a subgranular structure of substantially equiaxed cells having an average as cast diameter of between about 20  $\mu\text{m}$  and about 80  $\mu\text{m}$ ,

said ingot having a density greater than 99.5% of theoretical density of the alloy in the as-cast condition, and having less than five ppm total oxygen content and less than one ppm oxygen as insoluble oxide.

2. An ingot according to claim 1 wherein the aspect ratio of the grains is between about one and about six hundred.

3. An ingot according to claim 1 having a diameter in excess of about 15 centimeters wherein the grain size is substantially uniform when viewed on a surface cut perpendicular to the longitudinal axis of the ingot.

4. An ingot according to claim 1 comprising an alloy having a liquidus/solidus temperature range between about 65° C. and about 150° C.

5. An ingot according to claim 1 having a hollow interior.

6. An ingot according to claim 1 comprising a nickel or cobalt based alloy containing at least about 50% nickel or cobalt, and between about 10% and 20% chromium.

7. An alloy according to claim 6 containing aluminum and titanium, and including one or more elements selected from the group consisting of niobium, molybdenum, tungsten, yttrium, tantalum, hafnium, zirconium, and vanadium.

8. A vacuum cast high strength iron, nickel, or cobalt-based alloy ingot having at least about 50% nickel or cobalt and between about 10% and about 20% chromium, said ingot further containing aluminum and titanium, and including one or more elements selected from the group consisting of niobium, molybdenum, tungsten, yttrium, tantalum, hafnium, zirconium, and vanadium, said ingot having a grain size between about ASTM 3 and 9 when viewed on a surface cut perpendicular to the longitudinal axis of the ingot, and having longitudinal grains having a length of between about 0.5 millimeter and about 25 millimeters when viewed on a surface cut parallel to the longitudinal axis of the ingot, said ingot having an oxygen content in the form of insoluble oxide of less than about one ppm, and having a density greater than 99.5% of theoretical density of the alloy in the as-cast condition.

9. An ingot according to claim 8 having a diameter in excess of about 15 centimeters wherein the grain size is substantially uniform when viewed on a surface cut perpendicular to the longitudinal axis of the ingot.

10. An ingot according to claim 1 which is formed by the steps of:

directing an electron beam onto a stick of the alloy to produce a series of fully molten drops, each of which falls onto the upper surface of the ingot being formed along a substantially fixed drip axis to produce, on the ingot's upper surface, a film-like spatter having a thickness of between 0.04 and 0.08 mm and a maximum surface dimension of between about 3.8 and 6.2 centimeters, moving such mold in which the ingot is being formed with respect to the drip axis at a rate which is high enough so that successive drops will impinge upon

**15**

different portions of the ingot's upper surface, but which is low enough to result in substantially even spreading of said drops on the upper surface of the ingot, substantially covering the same with a series of spatters and building up the ingot vertically by successive drop impingements, and maintaining the melt rate such that the average rate of vertical buildup of the ingot is less than or equal to about one centimeter per minute.

**11.** The ingot of claim **10** wherein the melt rate is maintained so that the average rate of vertical buildup of the ingot is less than or equal to about one centimeter per minute, and the time interval between successive drop impingements in any given area is no more than about 60 seconds.

**16**

**12.** The ingot of claim **11**, wherein the pattern of successive drop impingements is sufficiently uniform to avoid localized pooling.

**13.** The ingot of claim **10**, wherein the mold is moved to form a series of substantially overlapping rings, each formed by moving the mold to a selected lateral position with respect to the drip axis, and rotating the mold substantially one revolution.

**14.** The ingot of claim **10**, wherein the melt rate is maintained such that the upper surface upon which the drops impinge is between about 28° C. and 110° C. below the solidus temperature of the alloy.

**15.** The ingot of claim **10**, wherein the ingot has a hollow interior by virtue of applying drops in an annular pattern.

\* \* \* \* \*

20

25

30

35

40

45

50

55

60

65